

1

2,860,996

## RUST PREVENTIVE COMPOSITION

Michael J. Furey, Berkeley Heights, N. J., assignor to  
Esso Research and Engineering Company, a corporation of Delaware

No Drawing. Application March 5, 1956  
Serial No. 569,253

6 Claims. (Cl. 106—14)

This invention relates to improved rust preventive compositions and, more particularly, to improved compositions having utility as solvent-cutback, hard film rust preventives. More specifically, the invention relates to asphalt cutback rust preventive compositions which have been stabilized against viscosity change during storage by inclusion therein of a minor proportion of a wax-substituted glyoxalidine.

Solvent-cutback, hard film rust preventives are known in the art. These are cold-applied compounds used for (1) the protection of metals exposed to a variety of outdoor weather conditions and (2) any general purpose preservation where a dry-to-touch film is desired. These materials generally contain an asphalt diluted with a petroleum solvent. The compounds are fluid in nature and may be applied to the metal surfaces to be protected by dipping, brushing or spraying. Upon evaporation of the solvent, a thin film, usually 0.002—0.004 inch thick, remains on the metal parts to serve as protection against weathering, corrosive fumes, and the like. In addition, the protective coating should not flow from the surfaces at high temperatures nor flake at low temperatures. When desired, the thin film is easily removed from the metal surfaces by the application of solvents such as petroleum solvents and the like.

Asphalts made by air-blowing or oxidation processes may be desirable as base materials for use in certain solvent-cutback, hard film rust preventives because these asphalts can be made to have a high softening point without being brittle at low temperatures. Accordingly, compounds based on these asphalts have less of a tendency to flow from metal surfaces in hot weather or to flake from metal surfaces when cold. However, solvent-cutback, hard film rust preventives made from these high softening point oxidized asphalts tend to increase in viscosity, thicken, and eventually gel on storage. This is particularly undesirable since the application of the rust preventive by dipping or spraying is made difficult or even impossible. Furthermore, the thickness of the film deposited upon the metal parts with the thickened or gelled material is considerably in excess of that desired.

It has now been found and forms the object of this invention that this undesirable thickening effect or gelling may be inhibited by the inclusion in these solvent-cutback, hard-film rust preventive compositions of a minor amount of a wax-substituted glyoxalidine compound.

The base material for the compositions of this invention comprises from 30 to 70% by weight of an asphalt and from 70 to 30% of a solvent therefor. The asphalt may be selected from the group of oxidized asphalts, or reduced and oxidized asphalts, with the former being preferred. Especially preferred are oxidized asphalts having a softening point between about 180° and 235° F.

The solvent used in preparing the base material may be any of the well-known petroleum solvents having flash points between about 100° and about 150° F. and mid-boiling points ranging from about 300° to about 350° F.

with a final boiling point below about 420° F. If it is desired, blends of various solvents may be made to use as the diluent for the asphaltic material.

The storage stability of asphalt cutbacks varies, to some extent, with (1) the concentration of asphalt (i. e., the more asphalt, the less stable), (2) the nature of the asphalt (oxidized asphalts gel more readily than straight reduced asphalts, and high softening point oxidized asphalts have the poorest stability), and (3) the nature of the solvent (e. g. cutbacks made with paraffinic solvents gel more than those made with aromatic solvents).

For adequate protection against corrosion under a wide variety of outdoor exposure conditions, the protective coating should be at least 0.002—0.004 inch thick. To accomplish this by a single dip or immersion of the metal in the rust-preventive, the concentration of the asphalt must be high enough (preferably 40—60%). At these concentrations, a serious storage stability problem exists. Storage stability with oxidized asphalts in the required concentration, would generally be:

- (1) Very, very poor with the more paraffinic solvents (e. g. hexane).
- (2) Better but still very poor with solvents containing about 20% aromatics.
- (3) Better yet with a highly aromatic and expensive solvent such as those containing in the neighborhood of 95% aromatics.

It is preferable to use as much paraffinic solvents as possible for economic reasons.

In accordance with the concept of the instant invention, the storage stability of all cutback asphalts from oxidized asphalts is improved without adversely affecting any other desirable properties of a good solvent-cutback rust preventive.

According to the invention cutback asphalts are blended with from 1 to 5 wt. percent of a wax-substituted glyoxalidine compound having the general formula:



wherein R is a monovalent saturated hydrocarbon radical having from 40 to 80 carbon atoms and wherein x is a number of from 1 to 2. A compound according to the formula above, when x is 1 and the average carbon content of the wax hydrocarbon radical R is 50, is available commercially under the trade name "Petrolite Wax Amine B."

In accordance with the concept of the instant invention, a solvent-cutback, hard film rust preventive base composition (Base A) was formulated from the following components:

(1) The asphalt used was an oxidized asphalt made by the pipe still reduction of Venezuelan (Lagunillas) Crude to 500/505° F. flash point stock followed by oxidation by air-blowing to 229° F. softening point. Its properties were as follows:

- (a) Penetration (cm.  $\times$  100) @:
  - 32° F. (200 g./60")—13
  - 77° F. (100 g./5")—21
  - 115° F. (50 g./5")—28
- (b) Ductility @ 77° F.—2.3 cm.
- (c) Pliability:
  - @ 0° F.—9°
  - @ 77° F.—118°
- (d) 99.90% soluble in carbon disulfide
- (e) 41.0% insoluble in 86° naphtha
- (f) 15.88% fixed carbon



What is claimed is:

1. The method of improving the storage stability of cutback asphalt-base thin film rust preventive compositions which comprises blending with said compositions a minor but viscosity-stabilizing amount of a wax amine compound having the formula



wherein R is a monovalent saturated hydrocarbon radical having from 40 to 80 carbon atoms and wherein x is a number of from 1 to 2.

2. A method according to claim 1 wherein said composition comprises a blend of from about 30 to 70 percent of an oxidized asphalt having a softening point between about 180° and 235° F. with from about 70 to 30 percent of a petroleum solvent naphtha.

3. A thin film rust inhibiting asphaltic composition consisting essentially of a cutback asphalt consisting of a blend of from about 30% to about 70% of an asphalt selected from the group consisting of oxidized asphalts and oxidized and reduced asphalts with from 70% to 30% by weight of a petroleum solvent inhibited against viscosity increase during storage with a minor but viscosity-stabilizing amount in the range of 1 to 5 weight percent of a wax amine compound having the formula



wherein R is a monovalent saturated hydrocarbon radical having from 40 to 80 carbon atoms and wherein  $x$  is a number of from 1 to 2.

- 10 4. A rust inhibiting composition according to claim 3  
5 wherein R is a monovalent saturated hydrocarbon radical containing about 50 carbon atoms and wherein  $x$  is 1.
  5. A rust inhibiting composition according to claim 3  
wherein from 1 to 5 wt. percent of the wax amine compound is used.
  - 10 6. A thin film rust inhibiting composition which consists of about 30% to about 70% by weight of an oxidized asphalt having a softening point between about 180° and 235° F. and about 70% to about 30% of a petroleum solvent naphtha having a final boiling point within the range of from 100° to 150° F. and a mid-boiling point within the range of from about 300° to 350° F. containing combined therein from 1.0 to 5.0 wt. percent of a wax glyoxalidine having the formula



- 25 wherein R is a monovalent saturated hydrocarbon radical containing about 50 carbon atoms and wherein  $x$  is 1.

**References Cited in the file of this patent**

UNITED STATES PATENTS

- 30 2,759,840 Crews et al. ----- Aug. 21, 1956  
2,766,132 Blair et al. ----- Oct. 9, 1956

## FOREIGN PATENTS

- 637,758 Great Britain ----- May 24, 1950

UNITED STATES PATENT OFFICE  
CERTIFICATE OF CORRECTION

Patent No. 2,860,996

November 18, 1958

Michael J. Furey

It is hereby certified that error appears in the printed specification of the above numbered patent requiring correction and that the said Letters Patent should read as corrected below.

Column 2, line 7, for "moree" read -- more --; column 6, line 14, for "final boiling" read -- flash --.

Signed and sealed this 9th day of June 1959.

(SEAL)

Attest:

KARL H. AXLINE  
Attesting Officer

ROBERT C. WATSON  
Commissioner of Patents